

# UNITED STATES PATENT OFFICE.

THOMAS H. STARTZMAN, OF TIFFIN, OHIO.

## IMPROVEMENT IN SOAP COMPOUNDS.

Specification forming part of Letters Patent No. **179,366**, dated June 27, 1876; application filed October 4, 1875.

*To all whom it may concern:*

Be it known that I, THOMAS H. STARTZMAN, of Tiffin, in the county of Seneca and State of Ohio, have invented a new and useful Soap Compound, which is fully described in the following specification.

This invention relates to that class of compounds called "soap-powder," used for washing clothes, &c.; and it consists in a composition formed by mixing together the following ingredients, in the manner and of the proportions as hereinafter set forth.

One gallon of rain-water, one pint of strong alcohol, four ounces of alum, eight ounces of aqua-ammonia, ten ounces of chemical soap, four pounds of borax, and ten pounds of sal-soda.

The chemical soap which I employ in this composition is one which I manufacture myself, and is composed of paraffine, nitrecine, beef's tallow, and common lye.

To prepare the composition the rain-water is put in a boiler over a slow fire; the chemical soap is then chipped or cut in small shavings and added thereto. As it dissolves add

the alum, borax, and sal-soda. The whole is then well stirred until dissolved, and then turned out into a vat and stirred until it is cold, when it is allowed to stand twenty-four hours. It is then placed again in the boiler, and as it melts the ammonia and alcohol are added, and the whole allowed to boil thirty minutes, stirring all the time. It is then turned out into the vat, and the stirring process continued until the whole mass is cold.

Having thus described my invention, what I claim is—

The hereinbefore-described soap compound, consisting of rain-water, alcohol, alum, aqua-ammonia, chemical soap, as herein specified, borax, and sal-soda, mixed in the proportions substantially as set forth and described.

In testimony that I claim the foregoing as of my own invention I hereby affix my signature in presence of two witnesses.

THOMAS H. STARTZMAN.

Witnesses:

G. I. KEEN,  
GEORGE HOSPELHAUN.